

June 13, 1944.

C. A. CROWLEY ET AL

2,350,991

BLUE PRINT SENSITIZER

Filed Aug. 16, 1941



## UNITED STATES PATENT OFFICE

2,350,991

## BLUEPRINT SENSITIZER

Clyde A. Crowley, Chicago, and George H. Good-year, Wilmette, Ill., assignors to The Huey Co., Chicago, Ill., a corporation of Illinois

Application August 16, 1941, Serial No. 407,162

21 Claims. (Cl. 95—6)

This application is a continuation in part of our application for patent on a Blueprint sensitizer filed September 27, 1939, Serial Number 296,768.

It has long been the desire of manufacturers of sensitized paper of the type called blueprint paper, to obtain a sensitizing which, when coated on paper, will give a sensitized sheet having the following characteristics:

1. The paper must have a high printing speed; that is, a short exposure will be sufficient to develop the desired color.

2. The exposed sheet must have an intense blue color, and clear whites to give the desired contrast.

3. When over-exposed, the blue color must be of good quality.

4. There must be no "bleeding" or running of color from the exposed portions into the unexposed white portions and white lines, even when the paper is badly over-exposed.

5. The sensitized paper must be capable of being stored under favorable conditions for periods up to two or three months, whereupon after development unexposed portions must contain a negligible amount of blue pigment.

For many years sensitizers have been formulated containing:

1. A light-sensitive ferric salt such as ferric ammonium citrate or ammonium ferrioxalate;

2. A ferricyanide salt; and,

3. Non-pigment-forming substances including other salts such as potassium oxalate, citrates, etc., which help keeping and washing properties, but do not themselves enter into the composition of the final pigment. In fact, their use in any amount decreases more or less the intensity and quality of the final blue pigment. When too much of non-pigment-forming substances is used, the color becomes unacceptable. Also, their presence markedly decreases the sensitivity of the paper to light.

In practice, the light-sensitive ferric compound has been used in great excess over the quantity which is chemically equivalent to the ferricyanide salt (customarily potassium ferricyanide). This is necessary to obtain sufficient light sensitivity. Ferricyanide is red in color and seems to filter out the shorter wave lengths of light which are most effective in causing the photochemical reaction. Therefore, to obtain high printing speed papers with this type of formulation, the stoichiometric ratio of potassium ferricyanide to reducible ferric iron must be very small. As ferricyanide is one of the essential components required to produce the final pigment, the maxi-

mum possible quantity of pigment, and hence the intensity of color possible, is limited by this component.

If a blueprint paper is even slightly over-exposed, ferrous iron in excess over the ferricyanide is formed, and in the development process this ferrous iron washes over into the unexposed portions, where it reacts with ferricyanide to form blue pigment. This is called "bleeding." Also, the presence of excess ferrous iron in the exposed portions adversely affects the quality of the blue pigment, giving it an undesirable slate or greyish cast. This is called "burning out."

If, in the sensitizer, the ratio of potassium ferricyanide to light-sensitive ferric compound is increased, the speed of the paper is decreased but the other desirable properties are gained in proportion. The sensitizers used by commercial blueprint paper manufacturers represent an unsatisfactory compromise between these inherent characteristics.

When a paper is exposed, the light-sensitive ferric compound must be reduced to a ferrous compound, and the ferricyanide salt is reduced to a ferrocyanide salt. These react to form insoluble ferroferrocyanide (ferrous ferrocyanide). Development consists of washing off the unexposed and excess chemicals, followed by the oxidation of the ferroferrocyanide to Prussian blue, and then washing off the excess oxidizing agent, which is usually potassium bichromate.

It has hitherto been suggested to use ferrocyanide salts in the sensitizer. When ferrocyanide was added to the customary formulation previously described, the following observations were made:

The speed of the paper was increased. However, in order to make it possible to wash the unexposed areas clean, it was necessary to add a much greater quantity of the non-pigment-forming substances such as oxalates, citrates, and phosphates to aid in washing and to use a substantial proportion of a ferricyanide salt. If the proportion of ferricyanide was decreased much below one-half the total quantity of iron-cyanides by weight, it was then necessary to add such a large proportion of non-pigment-forming substances as solubilizing agents that the quality of the final blue pigment was seriously impaired and the speed was reduced. When ferrocyanides were used in equal amount with the ferricyanide, the necessary amount of non-pigment-forming substances for solubilizing markedly desensitized the paper. The result was that it seemed impossible to add more than a certain limited amount of ferrocyanide because the addition of greater quantities required additional ferricyanide which

made the paper so slow it was not acceptable in commercial practice. If large quantities of non-pigment-forming substances were used instead of ferricyanide, the quality of color was greatly impaired.

The chemicals which actually enter into the formation of pigment in a blueprint paper are:

(1) light-sensitive ferric compounds such as ammonium ferrioxalate (ferric ammonium oxalate), sodium ferrioxalate, sodium iron tartrate, ferric ammonium citrate, or ferric potassium tartrate; and (2) iron-cyanogen compounds, which have in the past generally been ferricyanides such as potassium ferricyanide, sodium ferricyanide, or sodium potassium ferricyanide, but which also include ferrocyanides such as potassium or sodium ferrocyanide. All other substances which are included in a blueprint sensitizer are "non-pigment-forming" substances. Among the classes of non-pigment-forming substances which have been added to blueprint sensitizers are included:

(1) buffering agents such as phosphates, borax, oxalates, and many other types of compounds; (2) substances which are added to improve washing of the paper, which can be described broadly as "solubilizing" agents since they tend to make the unreacted pigment-forming chemicals more readily removable from the paper in washing; these include sugars, such as dextrose or sucrose, oxalates, phosphates, citrates, and many others; (3) oxidizing agents such as nitrites and chlorates, which frequently serve no apparent purpose, although in the case of papers containing ferrocyanides they will tend to increase ferricyanide at the expense of ferrocyanide; (4) binders, such as gums, starch, and the like, which are intended to prevent the sensitizer from soaking into the paper; (5) wetting agents, which are added primarily to aid in securing an even coat, but which may also aid in washing. This list by no means exhausts the tally of non-pigment-forming substances which have been proposed or used in blueprint papers. Some of these non-pigment-forming substances, as shown above, perform some useful function; e. g., buffer action or "solubilizing"; however, in many instances, the non-pigment-forming substances must be regarded as inert from every aspect. In either case, the non-pigment-forming substances are completely inert so far as forming pigment is concerned; and when used in excessive quantities, they are deleterious to the quality of the paper. Their deleterious effect arises from two sources; first, they interfere with the light reaction and reduce the speed of the paper, perhaps because they attenuate the pigment-forming substances as well as screening them from the light; and second, their presence in the pigmented areas after exposure imparts a dull, lifeless quality to the blue pigment in contrast to the brilliant blue formed when non-pigment-forming substances are absent or present only in moderate quantity.

Our invention consists of the discovery that when large quantities of ferrocyanide are used, approaching or exceeding the amount necessary for chemical equivalence to the light-sensitive iron compound, no ferricyanide salt is necessary to make the paper stable to storage, nor must such excessive amounts of non-pigment-forming substances, including washing or solubilizing agents, be present that the quality of the final

blue pigment is impaired. "Bleeding" and "burn-out" do not occur. Ferricyanide salts may be used if desired, but only as a control over the printing speed of the paper, since sensitizers formulated with the above components only can be made so fast that they cannot generally be used in the usual present day commercial blueprinting practice.

Relatively small amounts of potassium ferri-cyanide exert a very large effect in reducing the printing speed of sensitized papers.

Chemical equivalence is defined as two atoms of ferric iron as light-sensitive ferric compound or compounds for each iron atom present as a ferrocyanide or ferricyanide salt. This is true because the final reaction product on the completely exposed paper is ferrous ferrocyanide  $Fe^{+2}[Fe(CN)_6]^{4-}$  or its equivalent. Under these conditions there can be no excess ferrous iron to cause "bleeding" or "burn-out." As a matter of practical experience, it has been found that when there is only about 60% of the ferrocyanide salt present necessary for chemical equivalence to the light-sensitive ferric compound, the highest speed papers so formed are substantially non-bleeding in commercial printing machines. This is probably caused by the fact that a proportion of the light-sensitive ferric compound is shielded from the light by chemicals and paper fibers between it and the exposing lights, so that a portion of the light-sensitive ferric iron is never reduced. For slower papers this ratio should be increased somewhat to secure non-bleeding papers. It has been found that the addition of small amounts of a ferricyanide salt to such a sensitizer slows down the sensitizer and adds approximately the additional quantity of iron-cyanide salt necessary to insure substantially non-bleeding papers at the slower printing speeds.

At this point we wish to make the following clear. When there is a sufficient quantity of ferrocyanide and ferricyanide salts present in the sensitizer to be chemically equivalent to the light-sensitive ferric iron compound present, there is no bleeding. Bleeding under such circumstances is impossible. Small reductions in this ratio of total ferrocyanide and ferricyanide salts to light-sensitive ferric compounds do not cause bleeding under conditions of present day commercial practice. As the ratio of these salts is further decreased, bleeding eventually occurs and becomes increasingly severe as the ratio of these salts is still further reduced. As the ratio of total ferricyanide and ferrocyanide salts to light-sensitive ferric iron compounds is decreased, it becomes necessary to add increasing quantities of non-pigment-forming substances for solubilizing, in order to insure complete washing of the unexposed areas and to make the papers stable in storage.

A sensitizer in which ferrocyanide salt only is used, and in which it constitutes 60% of the quantity chemically equivalent to the light-sensitive ferric compound present, is approximately the practical boundary for substantially non-bleeding papers. When less than this ratio of ferrocyanide is used, without ferricyanide salts being present, the required quantity of non-pigment-forming substances required for solubilizing becomes excessive.

If ferricyanide is added to the sensitizer in addition to ferrocyanide, the ratio of iron-cyanides to ferric iron salts required for papers that are substantially non-bleeding in practice is greater. For slower papers in which ferri-

cyanide salts form an appreciable part, for example, from about 1% to about 5% by weight, of the iron-cyanide salts, a total content of iron-cyanide salts equivalent to 72% of the light-sensitive ferric compounds present is the practical minimum for substantially non-bleeding papers. If less than this quantity of ferrocyanide and ferricyanide combined is used, the papers will bleed; and, in addition, excessive amounts of non-pigment-forming substances are required to aid in washing, which reduce the speed of the paper and impair the quality of the blue pigment.

It has been found that the pH of these sensitizing solutions is not critical between reasonable limits. The pH must not be so high as to precipitate the iron from the light-sensitive ferric compound as ferric hydroxide or basic ferric compounds. This pH varies with the nature and quantity of the solubilizing salts present, being in general lower in the presence of phosphates and higher in the presence of citrates. A pH of 8.5 or 9.0 is approximately the upper limit.

When the pH is much below 4.0, it becomes more difficult to stabilize the paper from the standpoint of shelf life; however, we do not wish to limit the practice of this invention, by any minimum pH value, as certain classes of blueprint papers falling within the definitions of this invention can be manufactured from sensitizers adjusted to pH values below a pH of 4.

Further evidence of the non-critical pH range is indicated by the following observations. The sensitizing coating has been washed, with distilled water, from satisfactory papers containing ferrocyanide salts. The pH of these washings has been found invariably to lie between a pH value of 5.5 and 6.9. In general, we have observed that regardless of the pH of the original sensitizing solution, the pH of washings removed from the sensitized sheet invariably falls between 5.5 and 6.9.

In order to illustrate diagrammatically the relationships among the three chemical compounds or their equivalents which actually enter into the formation of the final blue pigment, the accompanying composition diagram has been prepared. These three compounds are considered to be 100% of the materials entering into the photochemical reaction. Non-pigment-forming substances which may be present are not considered. The specific compounds represented in the diagram are potassium ferrocyanide,  $K_4Fe(CN)_6 \cdot 3H_2O$ ; potassium ferricyanide,  $K_3Fe(CN)_6$ ; and ammonium ferrioxalate,  $(NH_4)_3Fe(C_2O_4)_3 \cdot 4H_2O$ .

as these are probably the most generally used. These materials are represented in actual weight percent. Any other combination of compounds such as sodium ferricyanide, ammonium ferrocyanide, and potassium iron tartrate may be applied to this diagram by using the corresponding chemically equivalent weights of the compounds used in plotting the diagram. Specific examples will be given later.

Any point within the triangle ABC represents a given composition of potassium ferrocyanide, potassium ferricyanide, and ammonium ferrioxalate. Point A represents 100% by weight of potassium ferricyanide. The farther from A a given point may be, the less potassium ferricyanide there will be in the sensitizer, until should the given point lie upon the side CB, the sensitizer would contain only potassium ferrocyanide and ammonium ferrioxalate. Lines with-

in the triangle and parallel to line CB represent a fixed percentage of compound A or potassium ferricyanide. These lines are drawn at 10% intervals. Likewise, point B represents 100% by weight of ammonium ferrioxalate



Lines parallel to side AC represent a given percentage of this compound. These lines are also shown at 10% intervals. Similarly, point C represents 100% by weight of potassium ferrocyanide



Lines parallel to side AB are drawn at 10% intervals to represent percentage of this compound.

Any sensitizer containing a ferrocyanide salt, or mixture of ferrocyanide salts, a ferricyanide salt or mixture of ferricyanide salts, and a light-sensitive ferric compound or mixture of light-sensitive ferric compounds is represented by some specific point on this diagram. Using this diagram, therefore, it is possible to compare specifically as regards content of pigment-forming chemicals any sensitizers whose active components are ferrocyanide, ferricyanide, and light-sensitive ferric compounds.

Point E represents that composition of potassium ferricyanide and ammonium ferrioxalate which contains a chemically equivalent quantity of ferrioxalate salt to light-sensitive ferric compound; that is, one iron atom from the ferricyanide salt to two iron atoms from the light-sensitive ferric compound. This point was calculated as follows:

35 Ammonium ferrioxalate



has a formula weight of 446 and contains one atomic weight of iron (55.84). Two formula weights of ammonium ferrioxalate (892) contain two atomic weights of iron. Potassium ferricyanide  $[K_4Fe(CN)_6 \cdot 3H_2O]$  has a formula weight of 329 and contains one atomic weight of iron. Therefore, 329 grams of potassium ferricyanide are chemically equivalent to 892 grams of ammonium ferrioxalate. See Table I.

Table I (Point E on diagram)

|                                    | Grams | Per cent |
|------------------------------------|-------|----------|
| $K_4Fe(CN)_6 \cdot 3H_2O$          | 329   | 27       |
| $(NH_4)_3Fe(C_2O_4)_3 \cdot 4H_2O$ | 892   | 73       |
|                                    | 1,221 | 100      |

55 Point D represents that composition of potassium ferrocyanide  $[K_4Fe(CN)_6 \cdot 3H_2O]$ , formula weight 422.33 and containing one atomic weight of iron, and ammonium ferrioxalate which contains a chemically equivalent quantity of ferrocyanide salt to light-sensitive ferric compound. See Table II for data.

Table II (Point D on diagram)

|                                    | Grams | Per cent |
|------------------------------------|-------|----------|
| $K_4Fe(CN)_6 \cdot 3H_2O$          | 422   | 32.2     |
| $(NH_4)_3Fe(C_2O_4)_3 \cdot 4H_2O$ | 892   | 67.8     |
|                                    | 1,314 | 100      |

60 Point F represents that composition of potassium ferrocyanide, potassium ferricyanide, and ammonium ferrioxalate which contains a quantity of ferrocyanide and ferricyanide salts to be chemically equivalent to the light-sensitive

ferric compound, and in which half the cyanide iron is contained in the ferricyanide salt and half in the ferrocyanide salt. See Table III.

Table III (Point F on diagram)

|                                                                                                    | Grams       | Per cent |
|----------------------------------------------------------------------------------------------------|-------------|----------|
| K <sub>3</sub> Fe(CN) <sub>6</sub> ·3H <sub>2</sub> O                                              | 422÷2=211   | 16.6     |
| K <sub>3</sub> Fe(CN) <sub>6</sub>                                                                 | 329÷2=164.5 | 13.0     |
| (NH <sub>4</sub> ) <sub>2</sub> Fe(C <sub>2</sub> O <sub>4</sub> ) <sub>2</sub> ·4H <sub>2</sub> O | 892         | 70.4     |
|                                                                                                    | 1,267.5     | 100      |

The straight line DFE on which these points D, E, and F lie represents all compositions of the above three compounds in which the iron-cyanide salts are chemically equivalent to the light-sensitive ferric compound and is, therefore, appropriately called the "non-bleed boundary." "Bleeding" cannot occur in sensitizers whose composition is represented by a point on this line or above and to the left of it. Line NPM, which is approximately parallel to the non-bleed boundary DFE, represents that composition of the above three compounds in which the total iron cyanide content is 72% of the quantity required to be chemically equivalent to the light sensitive ferric compound present. This is approximately the practical boundary for substantially non-bleeding papers, except for very fast papers containing a very low percentage of ferricyanide, where the percent of iron cyanide may be somewhat lower.

Points N and M represent respectively 72% chemical equivalence of potassium ferrocyanide and of potassium ferricyanide to ammonium ferrioxalate; therefore the mass of potassium ferricyanate present at point M is  $(0.72 \times 329)$  or 236 g. for a mass of 892 g. of ammonium ferrioxalate. Similarly at point N the composition is  $(0.72 \times 422)$  or 304 g. of potassium ferrocyanide for a mass of 892 g. of ammonium ferrioxalate. Point P represents a composition in which total iron-cyanides are 72% of an amount chemically equivalent to light-sensitive ferric compounds, and in which 50 mol percent of the iron-cyanides are present as ferrocyanide, and 50 mol percent as ferricyanide. Therefore ferricyanides and ferrocyanides are each 36% chemically equivalent to the light-sensitive ferric compound, from which the relative masses of the respective components readily can be computed.

Point L represents a composition containing equimolar quantities of potassium ferrocyanide and potassium ferricyanide, and containing no light-sensitive ferric compounds. It lies on the inside AC of the composition triangle. All sensitizers in which 50 mol percent of the iron cyanide compounds are present as ferrocyanides lie on the line LP. The area NPLC, therefore, includes all sensitizers in which the total content of iron-cyanides equals or exceeds 72% of chemical equivalence to the light-sensitive ferric compounds present, and in which the major portion (over 50 mol percent) of the iron-cyanides are present as ferrocyanides.

Point J represents a composition in which the ferrocyanide content is 60% of the quantity required to be chemically equivalent to the light-sensitive ferric compound present, and in which there is no ferricyanide. The line (AKJ) drawn from this point to A, of which JK is a segment, includes all sensitizers in which ferrocyanide content is 60% of the quantity required to be chemically equivalent to the light-sensitive ferric compound present. Point K represents a composition in which the ferrocyanide content is 60%

of the quantity required to be chemically equivalent to the light-sensitive ferric compound present, and the quantity of ferricyanide is equal to 48% of the quantity required to be chemically equivalent to the light-sensitive ferric compound present. Papers in which the quantity of ferrocyanide is greater than that represented by the line JK, and the quantity of ferricyanide is less than that represented by the line KC, are found to be substantially non-bleeding in practice, and the quantity of non-pigment-forming substances required for solubilizing is not excessive. These sensitizers are included in the area JKC. In all sensitizers included in this area, the major portion of the iron-cyanide compounds are present as ferrocyanide.

The following examples serve to illustrate our invention, although it is to be understood that they are merely examples and no unnecessary limitations are to be assumed therefrom.

Example I (Point 14)

|                                                                                                             |         |       |
|-------------------------------------------------------------------------------------------------------------|---------|-------|
| 1. Potassium oxalate (K <sub>2</sub> C <sub>2</sub> O <sub>4</sub> ·H <sub>2</sub> O)                       | g       | 8.76  |
| 2. Potassium carbonate (K <sub>2</sub> CO <sub>3</sub> ·2H <sub>2</sub> O)                                  | g       | 5.53  |
| 3. Potassium ferrocyanide                                                                                   | g       | 24.00 |
| 4. Ammonium ferrioxalate                                                                                    | g       | 24.00 |
| 5. Water to Baumé degrees                                                                                   | ml      | 14.5  |
| Volume                                                                                                      | ml      | 278   |
| Percent equivalence of total iron-cyanide compounds to light-sensitive ferric compounds                     | percent | 216   |
| Mass ratio of non-pigment forming substances to iron-cyanide compounds calculated as potassium ferrocyanide |         | 0.60  |

Example I is a sensitizer containing equal parts by weight of ammonium ferrioxalate and potassium ferrocyanide, and is represented as the midpoint on the line BC.

Instead of using potassium oxalate and potassium carbonate in preparing this sensitizer, and other sensitizers shown as examples hereafter, it is equivalent to use an amount of oxalic acid chemically equivalent to the potassium oxalate shown, and sufficient potassium carbonate to react with the oxalic acid and leave the amount of excess potassium carbonate shown. This is a common practice in the industry and is fully equivalent for every purpose, since the important factor is not what substances are used in making the sensitizer, but what substances are actually laid down on the paper, and in what quantity they are present. In Example I, the use of 6.00 g. of oxalic acid (H<sub>2</sub>C<sub>2</sub>O<sub>4</sub>·2H<sub>2</sub>O) and a total of 13.81 g. of potassium carbonate (K<sub>2</sub>CO<sub>3</sub>·2H<sub>2</sub>O) is equivalent to the use of 8.76 g. of potassium oxalate (K<sub>2</sub>C<sub>2</sub>O<sub>4</sub>·H<sub>2</sub>O) and 5.53 g. of potassium carbonate; and the reaction between 6.00 g. of oxalic acid and 13.81 g. of potassium carbonate will actually form in the sensitizing solution the same amounts of potassium oxalate, and carbonate ions as the solution of 8.76 g. of potassium oxalate and 5.53 g. of potassium carbonate; with the additional evolution in the case of the reaction between oxalic acid and potassium carbonate of carbon dioxide and the formation of water, neither of which will affect the composition of the sensitizer. It will be understood in the examples which follow that the same process of forming the actual non-pigment-forming substances desired in the sensitizing solution by chemical reaction from other substances can be applied.

The sensitizing solutions of Example I and the

examples which follow can be used at the concentration shown and will give good results if so used; or if desired they can be used at greater or lower concentration, within the limits of solubility of the components of the sensitizer at the coating temperature. So far as the characteristics of non-bleeding and freedom from burnout are concerned, the actual concentration of pigment-forming and non-pigment-forming substances is immaterial so long as the mass ratio of non-pigment-forming substances to iron-cyanide compounds, and the percent chemical equivalence of iron-cyanide compounds to light-sensitive ferric compounds are kept within the non-bleed limits shown in this specification.

#### Example II

Point 15 represents the following formula:

|                                                                                                       |         |      |
|-------------------------------------------------------------------------------------------------------|---------|------|
| 1. Potassium oxalate                                                                                  | g.      | 8.76 |
| 2. Potassium carbonate                                                                                | g.      | 4.97 |
| 3. Potassium ferrocyanide                                                                             | g.      | 18   |
| 4. Ammonium ferrioxalate                                                                              | g.      | 27   |
| 5. Water, to Baumé                                                                                    | degrees | 14.5 |
| Volume                                                                                                | cc.     | 290  |
| Percent equivalence of iron-cyanide compounds to light sensitive ferric compounds                     | percent | 141  |
| Mass of non-pigment-forming substances to iron-cyanide compounds calculated as potassium ferrocyanide |         | 0.76 |

Papers sensitized with this formula are so excessively fast that they cannot be used in the customary commercial blueprinting machine.

#### Example III

Point 16 represents the same formula as point 15 except that 3.82 g. of potassium ferricyanide were added. This paper has a printing speed about the same as the usual slow commercial papers. The total iron-cyanide content is equivalent to 22.90 g. calculated as potassium ferrocyanide; iron-cyanide compounds are 179% equivalent to light-sensitive ferric compounds, and the mass ratio of non-pigment-forming substances to total iron-cyanide compounds calculated as potassium ferrocyanide is 0.60.

Point 16 illustrates another convenient characteristic of this type of diagram. This point lies on a line drawn through A and point 15. Any point lying on this line has a constant ratio of ammonium ferrioxalate to potassium ferrocyanide, namely 27 to 18 or 3 to 2. In general, any line drawn through one vertex of the composition triangle represents a constant ratio of the components represented by the remaining two vertices.

#### Example IV

Point 17 locates the following formula on the composition triangle:

|                                                                                                             |         |      |
|-------------------------------------------------------------------------------------------------------------|---------|------|
| 1. Potassium oxalate                                                                                        | g.      | 6.35 |
| 2. Oxalic acid                                                                                              | g.      | 0.26 |
| 3. Potassium ferrocyanide                                                                                   | g.      | 18.0 |
| 4. Sodium ferrioxalate                                                                                      | g.      | 30.0 |
| 5. Potassium ferricyanide                                                                                   | g.      | 0.75 |
| 6. Water to make                                                                                            | cc.     | 300  |
| Percent equivalence of iron-cyanide compounds to light-sensitive ferric compounds                           | percent | 146  |
| Mass ratio of non-pigment-forming substances to iron-cyanide compounds calculated as potassium ferrocyanide |         | 0.35 |

Thirty g. of sodium ferrioxalate are equivalent to

$$30 \times \frac{446}{488} = 27.4 \text{ g.}$$

5 of ammonium ferrioxalate.

#### Example V

Point 18 represents the following formula:

|                           |         |      |
|---------------------------|---------|------|
| 1. Potassium carbonate    | g.      | 5.03 |
| 2. Potassium oxalate      | g.      | 8.76 |
| 3. Potassium ferrocyanide | g.      | 15.0 |
| 4. Ammonium ferrioxalate  | g.      | 30.0 |
| 5. Water to Baumé         | degrees | 14.5 |

Percent chemical equivalence of iron-cyanide compounds to light-sensitive ferric compounds percent 106

Mass ratio of non-pigment-forming substances to iron-cyanide compounds calculated as potassium ferrocyanide 0.91

#### Example VI

The formula represented by point 19 is the same as Example V with the addition of:

25 Potassium ferricyanide g. 0.375  
Percent chemical equivalence of iron-cyanide compounds to light-sensitive ferric compounds is 109%.

30 Mass ratio of non-pigment-forming substances to iron-cyanide compounds calculated as potassium ferrocyanide is 0.88.

#### Example VII

35 Point 20 represents the following formula:

|                           |         |       |
|---------------------------|---------|-------|
| 1. Potassium oxalate      | g.      | 10.97 |
| 2. Potassium carbonate    | g.      | 1.66  |
| 3. Potassium ferrocyanide | g.      | 15.00 |
| 4. Potassium ferricyanide | g.      | 0.75  |
| 40 5. Sodium ferrioxalate | g.      | 21.00 |
| 6. Ammonium ferrioxalate  | g.      | 3.75  |
| 7. Water to Baumé         | degrees | 14.5  |

Percent chemical equivalence of iron-cyanide compounds to light-sensitive ferric compounds Percent 147

45 Mass ratio of non-pigment-forming substances to iron-cyanide compounds calculated as potassium ferrocyanide 0.79

50 21 g. of sodium ferrioxalate are equivalent to

$$(21.00 \times \frac{446}{488})$$

55 or 19.20 g. of ammonium ferrioxalate. Therefore, the sensitizer contains the equivalent of (19.20 plus 3.75) or 22.95 g. of light-sensitive ferric compounds calculated as ammonium ferrioxalate.

Papers coated with these sensitizers are extremely fast.

The following is given as an example of the way by which other ferricyanide salts, ferrocyanide salts, and light-sensitive compounds than those shown on the diagram may be plotted on the diagram. The chemicals and quantities present which may eventually enter into the formation of pigment are as follows:

|                                     |    |       |
|-------------------------------------|----|-------|
| 1. Iron potassium tartrate (ferric) | g. | 30    |
| 2. Ammonium ferrocyanide            | g. | 11.35 |
| 70 3. Sodium ferricyanide           | g. | 8.65  |

1.  $K(FeO)C_4H_4O_6$  (formula weight 259 which contains one atomic weight of iron).

$$30 g. \times \frac{446}{259} = 51.7 \text{ g.}$$

of ammonium ferrioxalate required to be chemically equivalent.

2.  $(\text{NH}_4)_2\text{Fe}(\text{CN})_6 \cdot 6\text{H}_2\text{O}$  (formula weight 392 which contains one atomic weight of iron).

$$11.35 \times \frac{422}{392} = 12.2 \text{ g.}$$

of potassium ferrocyanide required to be chemically equivalent.

3.  $\text{Na}_3\text{Fe}(\text{CN})_6 \cdot 3\text{H}_2\text{O}$  (formula weight 299 which contains one atomic weight of iron).

$$8.65 \times \frac{329}{299} = 9.2 \text{ g.}$$

potassium ferricyanide required to be chemically equivalent.

Table IV indicates the calculations required to plot the point.

Table IV

|                                                                      | Grams | Per cent |
|----------------------------------------------------------------------|-------|----------|
| 1. $(\text{NH}_4)_2\text{Fe}(\text{CN})_6 \cdot 4\text{H}_2\text{O}$ | 51.7  | 70.6     |
| 2. $\text{K}_4\text{Fe}(\text{CN})_6 \cdot 3\text{H}_2\text{O}$      | 12.2  | 16.7     |
| 3. $\text{K}_4\text{Fe}(\text{CN})_6$                                | 9.2   | 12.7     |
|                                                                      | 73.1  | 100.0    |

This is approximately point F.

Excellent results are obtained by employing compositions in the area near the non-bleed boundary DFE and the line CB and a particularly important, though limited, embodiment of our invention comprises compositions falling within the shaded area on the figure of the drawing and wherein the weight of non-pigment-forming substances, such as buffering agents, solubilizing agents, washing aids, and the like is not in excess of 1.5 times the weight of all of the iron-cyanide salts or compounds calculated as potassium ferrocyanide ( $\text{K}_4\text{Fe}(\text{CN})_6 \cdot 3\text{H}_2\text{O}$ ) and is preferably equal in weight to or less than the weight of the said iron-cyanide compounds calculated as potassium ferrocyanide. For best results, the total iron-cyanide salt content is at least 80% of that quantity required to be chemically equivalent to the light-sensitive ferric compound or compounds. The ferricyanide salt may, for example, comprise from 2% to 27% by weight of the total of the ferrocyanide salt and ferricyanide salt, a more restricted range being up to 6% and a particularly desirable and especially satisfactory range being from about 1% to about 5% or 6%. The ferrocyanide should comprise from 25% to 27% by weight of the total pigment-forming substances in the particularly preferred sensitizers of our invention. The following examples represent a series of sensitizers which are unusually efficacious and which are shown on the diagram as points 8 to 12, inclusive.

|                                                                                                             | Point No. |       |       |       |       |
|-------------------------------------------------------------------------------------------------------------|-----------|-------|-------|-------|-------|
|                                                                                                             | 8         | 9     | 10    | 11    | 12    |
| <b>Example...</b>                                                                                           |           |       |       |       |       |
| 1. Potassium oxalate                                                                                        | grams     | 10.92 | 10.92 | 10.92 | 10.92 |
| 2. Potassium carbonate                                                                                      | do        | 3.93  | 3.93  | 3.93  | 3.93  |
| 3. Potassium ferrocyanide                                                                                   | do        | 15.00 | 15.00 | 15.00 | 15.00 |
| 4. Potassium ferricyanide                                                                                   | do        | 0.00  | 0.66  | 1.13  | 1.88  |
| 5. Ammonium ferrioxalate                                                                                    | do        | 41.00 | 41.00 | 41.00 | 41.00 |
| 6. Water to Baumé                                                                                           | degrees   | 19    | 19    | 19    | 19    |
| Volume                                                                                                      | ml.       | 275   | 275   | 275   | 275   |
| Percent chemical equivalence of iron-cyanide compounds to light-sensitive ferric compounds                  | percent   | 77.3  | 81.2  | 84.8  | 89.7  |
| Mass ratio of non-pigment-forming substances to iron-cyanide compounds calculated as potassium ferrocyanide |           | 0.99  | 0.94  | 0.90  | 0.85  |
|                                                                                                             |           |       |       |       | 0.79  |

Example VIII represents the basic solution and contains no ferricyanide salt, as the position of point 8 on the side CB indicates.

Examples IX to XII represented by points 9 to 12 inclusive are formed by adding quantities of ferricyanide salt to the basic sensitizer represented by point 8. Therefore, all these points lie on a straight line passing through point A.

Paper sensitized by the formula given as Example IX and represented by point 9 is exceptionally fast and should, therefore, be used under conditions which take this factor into account.

Points 10, 11 and 12 represent sensitizers which, as indicated hereinabove, are especially satisfactory. These cover a rapid speed range but are readily adapted to present day commercial equipment. Due to non-bleeding and lack of burn-out, in general, they produce faster printing papers than those produced with the older type of sensitizers containing no ferrocyanide salt. When the customary exposure for the older type is given to these newer papers, a much deeper blue color is obtained without danger of "bleeding" or of "burn-out."

Examples XIII to XVII, inclusive show the effect of increasing greatly the excess of iron-cyanide compounds over light-sensitive ferric iron compounds.

|                                                                                                             | Example XIII<br>(point 31) | Example XIV<br>(point 32) | Example XV<br>(point 33) |
|-------------------------------------------------------------------------------------------------------------|----------------------------|---------------------------|--------------------------|
| Potassium oxalate                                                                                           | grams                      | 20.84                     | 20.84                    |
| Potassium carbonate                                                                                         | do                         | 7.86                      | 7.86                     |
| Potassium ferrocyanide                                                                                      | do                         | 37.90                     | 37.90                    |
| Ammonium ferrioxalate                                                                                       | do                         | 20.00                     | 20.00                    |
| Potassium ferricyanide                                                                                      | do                         | 3.54                      | 29.50                    |
| Water to Baumé                                                                                              | degrees                    | 16.5                      | 15.5                     |
| Percent equivalence of iron-cyanide compounds to light-sensitive ferric compounds                           | percent                    | 400                       | 448                      |
| Mass ratio of non-pigment-forming substances to iron-cyanide compounds calculated as potassium ferrocyanide |                            | 0.78                      | 0.70                     |
|                                                                                                             |                            |                           | 0.39                     |

|                                                                                                             | Example XVI<br>(point 34) | Example XVII<br>(point 35) |       |
|-------------------------------------------------------------------------------------------------------------|---------------------------|----------------------------|-------|
| Potassium oxalate                                                                                           | grams                     | 20.84                      | 20.84 |
| Potassium carbonate                                                                                         | do                        | 7.86                       | 7.86  |
| Potassium ferrocyanide                                                                                      | do                        | 18.96                      | 28.40 |
| Ammonium ferrioxalate                                                                                       | do                        | 20.00                      | 20.00 |
| Potassium ferricyanide                                                                                      | do                        | 14.75                      | 7.38  |
| Water to Baumé                                                                                              | degrees                   | 13.9                       | 16.1  |
| Percent equivalence of iron-cyanide compounds to light-sensitive ferric compounds                           | percent                   | 400                        | 400   |
| Mass ratio of non-pigment-forming substances to iron-cyanide compounds calculated as potassium ferrocyanide |                           | 0.78                       | 0.78  |

Example XV contains ferrocyanide and ferricyanide 800% of an amount that would be chemically equivalent to the light-sensitive ferric compounds present. Although this paper is quite slow because of the high concentration of ferricyanide, it is, nevertheless, a usable paper, washes readily and gives non-bleeding prints free from burnout. The mass ratio of non-pigment-forming substances to total iron-cyanide compounds calculated as potassium ferrocyanide is only 0.39 in this sensitizer. Example XIII is a high-speed paper with good color, with good washing characteristics, non-bleeding, and free from burnout. Examples XIV and XVII are somewhat slower but still well within the speed range of commercial papers. Example XVI is somewhat slower than most commercially used papers, but gives excellent prints, and with Example XV il-

lustrates the range of compositions which give non-bleeding papers.

The compositions of pigment-forming chemicals which are required to form non-bleeding papers with the major portion of their iron-cyanide compounds present as ferrocyanide are represented by the following areas on the diagram:

(1) The non-bleed region DFLC, which is bounded by the segment DF of the non-bleed boundary, the line FL, and the sides AC and BC of the composition triangle. Sensitizers included in this area contain an amount of iron-cyanides at least chemically equivalent to the light-sensitive ferric compounds present, and contain ferrocyanides as the major pigment-forming iron-cyanide compound. Papers prepared from sensitizers represented by points within this area cannot bleed, because it is not possible to form free ferrous iron over an amount chemically equivalent to the iron-cyanide compounds present.

(2) The area NPLC, which includes all sensitizers containing iron-cyanides in amounts 72% or more of the quantity chemically equivalent to the light-sensitive ferric compounds present, and containing less than 50 molal percent of their iron-cyanide content as ferricyanide. (This is less than 43.8% of the iron-cyanide compounds as ferricyanides on a mass percent basis, if the ferrocyanide and ferricyanide are both present in their entirety as the potassium salts.) Such sensitizers contain ferrocyanide salts as the major pigment-forming iron-cyanide compound, and are substantially non-bleeding in practice without the necessity of loading the sensitizer with non-pigment-forming substances to secure satisfactory washing or other characteristics.

(3) The area JKC, which includes all sensitizers with content of ferrocyanides 60% or more of the amount chemically equivalent to the light-sensitive ferric compounds present, and ferricyanide content less than 48% of an amount equivalent chemically to the light-sensitive ferric compounds present. Papers sensitized with such sensitizers are substantially non-bleeding in practice without the necessity of loading the sensitizers with non-pigment-forming substances to secure satisfactory washing. In these sensitizers, ferrocyanide salts are the predominant pigment-forming cyanide compounds present.

All papers containing an excess of iron-cyanide compounds over light-sensitive ferric salts are non-bleeding, no matter how large the excess of iron-cyanide compounds may be. We have shown formulas for non-bleeding papers containing ferrocyanide salts up to 400% (Example XIII) of the amount equivalent to light-sensitive ferric compounds present, which are usable in present commercial practice. Example XV contains total iron-cyanide compounds 800% of the amount chemically equivalent to light-sensitive ferric compounds present. Further increases in the ratio of iron-cyanide salts to light-sensitive ferric salts will continue to give non-bleeding papers. At present there is no commercial advantage in using such papers, particularly because the excess ferrocyanide cannot at present be utilized; however, such papers are usable and will give prints free from bleeding.

Curved lines *a*, *b*, *c*, *d* represent approximately equal speed lines. Sensitizers whose composition is represented by points along any one of these lines all have approximately the same printing speed. The curve to the right at the lower portion of these lines is probably due to the

desensitizing effect of the solubilizing salts which are required in much large concentration in this region as previously discussed. These lines are appropriately called iso-speed lines.

5 It has been explained heretofore that potassium ferrocyanide, potassium ferricyanide, and ammonium ferrioxalate are used as examples in the description of the accompanying chart, and that other compounds may be used in place thereof, in quantities that will provide corresponding chemically equivalent weights, and this is contemplated in the accompanying claims.

We claim:

1. A sensitizer for blueprint papers and the like, containing a ferrocyanide salt, a ferricyanide salt, a light-sensitive ferric compound, and non-pigment-forming substances, in which the total iron-cyanide content is at least 72% of that quantity required to be chemically equivalent to the light-sensitive ferric compound, and in which the ferricyanide content is less than 50 molal percent of the total content of iron-cyanide compounds, and in which the weight of non-pigment-forming substances is not more than 1.5 times the weight of all iron-cyanide compounds, calculated as potassium ferrocyanide.

2. A blueprint paper having a sensitizer thereon containing a ferrocyanide salt, a ferricyanide salt, a light-sensitive ferric compound, and non-pigment-forming substances, in which the total iron-cyanide content is at least 72% of the quantity required to be chemically equivalent to the light-sensitive ferric compound, and in which the ferricyanide content is less than 50 molal percent of the total content of iron-cyanide compound, and in which the weight of non-pigment-forming substances is not more than 1.5 times the weight of all iron-cyanide compounds, calculated as potassium ferrocyanide.

3. A method of making blueprints, which consists in coating paper or the like with a sensitizer containing a ferrocyanide salt, a ferricyanide salt, a light-sensitive ferric compound, and non-pigment-forming substances in which the total iron-cyanide content is at least 72% of that quantity required to be chemically equivalent to the light-sensitive ferric compound, and in which the ferricyanide content is less than 50 molal percent of the total content of iron-cyanide compounds, and in which the weight of non-pigment-forming substances is not more than 1.5 times the weight of all iron-cyanide compounds, calculated as potassium ferrocyanide; exposing said paper under a design to light, and then developing and washing said paper.

4. A sensitizer for blueprint paper and the like containing a ferrocyanide salt, a ferricyanide salt, and a light-sensitive ferric compound, the said composition falling within the area DFLC on the figure of the drawing when calculated as  $K_4Fe(CN)_6 \cdot 3H_2O$ ,  $K_3Fe(CN)_6$ , and



wherein the points defining said area have the following compositions by weight:

| Point | $K_4Fe(CN)_6 \cdot 3H_2O$ | $K_3Fe(CN)_6$        | $(NH_4)_3Fe(C_2O_4)_3 \cdot 4H_2O$ |
|-------|---------------------------|----------------------|------------------------------------|
| D     | Percent<br>32.8<br>16.6   | Percent<br>0<br>13.0 | Percent<br>67.8<br>70.4            |
| F     | 58.2                      | 43.8                 | 0                                  |
| L     | 100                       | 0                    | 0                                  |
| C     |                           |                      |                                    |

5. A sensitizer for blueprint paper and the like containing a ferrocyanide salt, a ferricyanide

salt, and a light-sensitive ferric compound, the said composition falling within the area NPLC on the figure of the drawing when calculated as  $K_4Fe(CN)_6 \cdot 3H_2O$ ,  $K_3Fe(CN)_6$ , and



wherein the points defining said area have the following compositions by weight:

| Point | $K_4Fe(CN)_6 \cdot 3H_2O$ | $K_3Fe(CN)_6$ | $(NH_4)_3Fe(C_2O_4)_3 \cdot 4H_2O$ |
|-------|---------------------------|---------------|------------------------------------|
|       | Percent                   | Percent       | Percent                            |
| N     | 25.4                      | 0             | 74.6                               |
| P     | 13.1                      | 10.2          | 76.7                               |
| L     | 56.2                      | 43.8          | 0                                  |
| C     | 100                       | 0             | 0                                  |

said sensitizer also containing non-pigment-forming substances the weight of which is not more than 1.5 times the weight of all iron-cyanide compounds calculated as  $K_4Fe(CN)_6 \cdot 3H_2O$ .

6. A sensitizer for blueprint paper and the like containing a ferrocyanide salt, a ferricyanide salt, and a light-sensitive ferric compound, the said composition falling within the shaded area on the figure of the drawing when calculated as  $K_4Fe(CN)_6 \cdot 3H_2O$ ,  $K_3Fe(CN)_6$ , and



said sensitizer also containing non-pigment-forming substances, the weight of which is not more than 1.5 times the weight of all iron-cyanide compounds calculated as  $K_4Fe(CN)_6 \cdot 3H_2O$ .

7. A sensitizer for blueprint paper and the like containing a ferrocyanide salt, a ferricyanide salt, and a light-sensitive ferric compound, the said composition falling within the area JKC on the figure of the drawing when calculated as  $K_4Fe(CN)_6 \cdot 3H_2O$ ,  $K_3Fe(CN)_6$ , and



wherein the points defining said area have the following compositions by weight:

| Point | $K_4Fe(CN)_6 \cdot 3H_2O$ | $K_3Fe(CN)_6$ | $(NH_4)_3Fe(C_2O_4)_3 \cdot 4H_2O$ |
|-------|---------------------------|---------------|------------------------------------|
|       | Percent                   | Percent       | Percent                            |
| J     | 22.1                      | 0             | 77.9                               |
| K     | 19.4                      | 12.1          | 68.5                               |
| C     | 100                       | 0             | 0                                  |

said sensitizer also containing non-pigment-forming substances the weight of which is not more than 1.5 times the weight of all iron-cyanide compounds calculated as  $K_4Fe(CN)_6 \cdot 3H_2O$ .

8. A sensitizer for blueprint papers and the like containing a ferrocyanide salt, a ferricyanide salt, a light-sensitive ferric compound, and non-pigment-forming substances, the quantity of ferricyanide salt comprising from 2% to 27% by weight of the total iron-cyanide salts in the composition, the total iron-cyanide salt content comprising at least 80% of that quantity required to be chemically equivalent to the light-sensitive ferric compound, and the weight of the non-pigment-forming substances being not in excess of the weight of all iron-cyanide salts calculated as  $K_4Fe(CN)_6 \cdot 3H_2O$ .

9. A sensitizer for blueprint papers and the like containing a ferrocyanide salt, a ferricyanide salt, a light-sensitive ferric compound, and non-pigment-forming substances, the quantity of ferricyanide salt comprising from 2% to 27% by weight of the total iron-cyanide salts in the composition, the total iron-cyanide salt content com-

prising at least 72% of that quantity required to be chemically equivalent to the light-sensitive ferric compound, and the weight of the non-pigment-forming substances being not in excess of 1.5 times the weight of all iron-cyanide salts calculated as  $K_4Fe(CN)_6 \cdot 3H_2O$ .

10. A sensitizer for blueprint papers and the like containing a ferrocyanide salt, a ferricyanide salt, a light-sensitive ferric compound, and non-pigment-forming substances, the quantity of ferricyanide salt comprising from about 1% to about 6% by weight of the total iron-cyanide salts in the composition, the total iron-cyanide salt content comprising at least 72% of that quantity required to be chemically equivalent to the light-sensitive ferric compound, and the weight of the non-pigment-forming substances being not in excess of 1.5 times the weight of all iron-cyanide salts calculated as  $K_4Fe(CN)_6 \cdot 3H_2O$ .

11. A non-bleeding blueprint paper having a storage life of at least one year under ordinary atmospheric conditions, said paper having a sensitizer thereon containing a ferrocyanide salt, a ferricyanide salt, a light-sensitive ferric compound, and non-pigment-forming substances, in which the total iron-cyanide salt content is at least 72% of the quantity required to be chemically equivalent to the light-sensitive ferric compound, the ferricyanide salt content being from 2% to 27% by weight of the total content of the ferrocyanide salt and the ferricyanide salt, and in which the weight of non-pigment-forming substances is not in excess of 1.5 times the weight of both the ferrocyanide salt and the ferricyanide salt together calculated as  $K_4Fe(CN)_6 \cdot 3H_2O$ .

12. A non-bleeding blueprint paper having a storage life of at least one year under ordinary atmospheric conditions, said paper having a sensitizer thereon containing an alkali ferrocyanide salt, an alkali ferricyanide salt, a light-sensitive ferric compound, and non-pigment-forming substances, in which the total iron-cyanide salt content is at least 80% of the quantity required to be chemically equivalent to the light-sensitive ferric compound, the alkali ferricyanide salt content being from 2% to 27% by weight of the total content of the alkali ferrocyanide salt and the alkali ferricyanide salt, and in which the weight of non-pigment-forming substances is not in excess of the weight of both the alkali ferrocyanide salt and the alkali ferricyanide salt together calculated as  $K_4Fe(CN)_6 \cdot 3H_2O$ .

13. A non-bleeding blueprint paper having a storage life of at least one year under ordinary atmospheric conditions, said paper having a sensitizer thereon containing an alkali metal ferrocyanide, an alkali metal ferricyanide, a light-sensitive ferric compound, and non-pigment-forming substances, in which the total iron-cyanide salt content is at least 72% of the quantity required to be chemically equivalent to the light-sensitive ferric compound, the alkali metal ferricyanide content being from about 1% to about 6% by weight of the total content of the alkali metal ferrocyanide and the alkali metal ferricyanide, and in which the weight of non-pigment-forming substances is not in excess of 1.5 times the weight of both the alkali metal ferrocyanide and the alkali metal ferricyanide together calculated as  $K_4Fe(CN)_6 \cdot 3H_2O$ .

14. A light-sensitive coated paper, said coating containing a ferrocyanide salt, a ferricyanide salt, a light-sensitive ferric compound, and non-pigment-forming substances, the coating composition falling within the shaded area on the

figure of the drawing when calculated as  $K_4Fe(CN)_6 \cdot 3H_2O$ ,  $K_3Fe(CN)_6$ ,



and the weight of the non-pigment-forming substances being not more than 1.5 times the weight of both the ferrocyanide salt and the ferricyanide salt together calculated as  $K_4Fe(CN)_6 \cdot 3H_2O$ .

15. A light-sensitive coated paper, said coating containing an alkali ferrocyanide salt, an alkali ferricyanide salt, a light-sensitive ferric compound, and non-pigment-forming substances, the coating composition falling within the shaded area on the figure of the drawing when calculated as  $K_4Fe(CN)_6 \cdot 3H_2O$ ,  $K_3Fe(CN)_6$ , and



the weight of the non-pigment-forming substances being not in excess of the weight of both the alkali ferrocyanide salt and the alkali ferricyanide salt together calculated as



16. A light-sensitive coated paper, said coating containing a ferrocyanide salt, a ferricyanide salt, a light-sensitive ferric compound as pigment-forming substances, and non-pigment-forming substances, the ferrocyanide comprising between 25% and 27% by weight of the total pigment forming substances, the ferricyanide salt comprising from about 1% to about 5% by weight of the pigment-forming substances, and the weight of the non-pigment-forming substances being not in excess of the weight of both the ferrocyanide salt and the ferricyanide salt calculated as  $K_4Fe(CN)_6 \cdot 3H_2O$ .

17. A light-sensitive coated paper, said coating containing a ferrocyanide salt, a ferricyanide salt, a light-sensitive ferric compound as pigment-forming substances, and non-pigment-forming substances, the ferrocyanide comprising between 25% and 27% by weight of the total pigment-forming substances, the ferricyanide salt comprising up to 6% by weight of the pigment forming substances, and the weight of the non-pigment-forming substances being not more than 1.5 times the weight of both the ferrocyanide salt and the ferricyanide salt together calculated as  $K_4Fe(CN)_6 \cdot 3H_2O$ .

18. A method of making blueprints which comprises coating paper or the like with a sensitizer containing a ferrocyanide salt, a ferricyanide salt, a light-sensitive ferric compound, and non-pigment-forming substances, said composition falling within the area DFLC on the figure of the drawing when calculated as  $K_4Fe(CN)_6 \cdot 3H_2O$ ,  $K_3Fe(CN)_6$ , and  $(NH_4)_3Fe(C_2O_4)_3 \cdot 4H_2O$ , wherein the points defining said area have the following compositions by weight:

| Point  | $K_4Fe(CN)_6 \cdot 3H_2O$ | $K_3Fe(CN)_6$ | $(NH_4)_3Fe(C_2O_4)_3 \cdot 4H_2O$ |
|--------|---------------------------|---------------|------------------------------------|
|        | Percent                   | Percent       | Percent                            |
| D..... | 32.8                      | 0             | 67.8                               |
| F..... | 16.6                      | 13.0          | 70.4                               |
| L..... | 56.2                      | 43.8          | 0                                  |
| C..... | 100                       | 0             | 0                                  |

exposing said coated paper under a design to light, washing, oxidizing, again washing, and then drying said paper.

19. A method of making blueprints and the

like which comprises coating paper or the like with a sensitizer containing a ferrocyanide salt, a ferricyanide salt, a light-sensitive ferric compound, and non-pigment-forming substances, said composition falling within the area NPLC on the figure of the drawing when calculated as  $K_4Fe(CN)_6 \cdot 3H_2O$ ,  $K_3Fe(CN)_6$ , and



10 wherein the points defining said area have the following compositions by weight:

| Point  | $K_4Fe(CN)_6 \cdot 3H_2O$ | $K_3Fe(CN)_6$ | $(NH_4)_3Fe(C_2O_4)_3 \cdot 4H_2O$ |
|--------|---------------------------|---------------|------------------------------------|
|        | Percent                   | Percent       | Percent                            |
| N..... | 25.4                      | 0             | 74.6                               |
| P..... | 13.1                      | 10.2          | 76.7                               |
| L..... | 56.2                      | 43.8          | 0                                  |
| C..... | 100                       | 0             | 0                                  |

20 the weight of the non-pigment-forming substances being not in excess of the weight of all iron-cyanide compounds calculated as



25 exposing said coated paper under a design to light, washing, oxidizing, again washing, and then drying said paper.

20. A method of making blueprints and the like which comprises coating paper or the like with a sensitizer containing a ferrocyanide salt, a ferricyanide salt, a light-sensitive ferric compound, and non-pigment-forming substances, said composition falling within the area JKC on the figure of the drawing when calculated as  $K_4Fe(CN)_6 \cdot 3H_2O$ ,  $K_3Fe(CN)_6$ , and



wherein the points defining said area have the following compositions by weight:

| Point  | $K_4Fe(CN)_6 \cdot 3H_2O$ | $K_3Fe(CN)_6$ | $(NH_4)_3Fe(C_2O_4)_3 \cdot 4H_2O$ |
|--------|---------------------------|---------------|------------------------------------|
|        | Percent                   | Percent       | Percent                            |
| J..... | 22.1                      | 0             | 77.9                               |
| K..... | 19.4                      | 12.1          | 68.5                               |
| C..... | 100                       | 0             | 0                                  |

the weight of the non-pigment-forming substances being not more than 1.5 times the weight of all iron-cyanide compounds calculated as

50  $K_4Fe(CN)_6 \cdot 3H_2O$ , exposing said coated paper under a design to light, washing, oxidizing, again washing, and then drying said paper.

21. A method of making blueprints and the like which comprises coating paper or the like with a sensitizer containing a ferrocyanide salt, a ferricyanide salt, a light-sensitive ferric compound, and non-pigment-forming substances, the said composition falling within the shaded area on the figure of the drawing when calculated as  $K_4Fe(CN)_6 \cdot 3H_2O$ ,  $K_3Fe(CN)_6$ , and



the weight of the non-pigment-forming substances being not in excess of all iron-cyanide compounds calculated as  $K_4Fe(CN)_6 \cdot 3H_2O$ , exposing said paper under a design to light, washing, oxidizing, again washing, and then drying said paper.

CLYDE A. CROWLEY.

GEORGE H. GOODYEAR.